

# UNITED STATES PATENT OFFICE.

WILLIAM FRIESE-GREENE, OF LONDON, ENGLAND.

## MANUFACTURE OF PAPER FOR ELECTRIC PRINTING.

SPECIFICATION forming part of Letters Patent No. 655,970, dated August 14, 1900.

Application filed March 13, 1900. Serial No. 8,443. (No specimens.)

*To all whom it may concern:*

Be it known that I, WILLIAM FRIESE-GREENE, photographer, of 39 King's road, Chelsea, London, England, have invented 5 certain new and useful Improvements in the Manufacture of Paper for Electric Printing, of which the following is a specification.

In my prior application for patent, Serial No. 733,130, filed October 10, 1899, for an improvement in paper, &c., I describe and claim, broadly, an article of manufacture such as paper or textile fabric containing a substance which will instantaneously form visible and permanent marks when an electrical current 15 is passed through the same in the presence of moisture. My present invention has reference to one specific variety of such paper and to the manufacture thereof, said paper being especially adapted for use in electrical inkless 20 printing.

The present invention consists in applying an extract, liquid, or solution of the character hereinafter described to the paper in the course of the manufacture of the latter. The 25 extract, liquid, or solution may be incorporated with pulp before its manufacture into paper or may be distributed, preferably in a state of fine division, upon the layer of pulp when on the wire web or other "former" before or during the "forming" of the paper, or 30 upon the paper after it has "formed," and either when still moist or after it has become dry. The said liquid or solution is an extract of marine algae and is obtained, preferably, as 35 follows:

I take sea-water and place therein an amount of a marine alga or marine algae, preferably seaweed—say one pound to the gallon—and add common washing soda—say one-fourth 40 of a pound per pound of weed. I boil the mixture until the liquor becomes clouded—say for about twenty-five minutes. This cloudiness is due to a substance of an alkaline nature in suspension. I then add, preferably after the liquor has cooled, sufficient 45 acid, hydrochloric by preference, to dissolve the clouding matter. I decant off the liquor and add to it hyposulphite of soda in the proportion of, say, one-fourth of a pound per gallon 50 of decanted liquor. I thus get the extract, liquid, or solution, which I incorporate with paper-pulp or distribute over the paper during or after forming, as hereinbefore explained. The finished paper shall contain 55 about five per cent. of the liquid or extract.

The proportions above specified are those which I have found to give the best results in practice; but it will be understood that I do not limit myself thereto.

Paper thus made will give an instantaneous 60 and permanent dark-brown print produced electrically thereon.

I have not yet ascertained the exact nature or composition of the liquid or solution obtained in the manner hereinbefore described, 65 nor am I at present certain as to what ingredient or ingredients of same are effective in electrical inkless printing. The present invention includes the use of the effective ingredient or ingredients in the manner described, whether produced as hereinbefore 70 described or in any other way.

What I claim, and desire to secure by Letters Patent, is—

1. The method or process of making paper 75 suitable for electric printing, which consists in treating paper with an extract of marine algae, substantially as described.

2. The method or process of making paper suitable for electric printing, which consists 80 in treating paper with an extract of seaweed, substantially as described.

3. In the manufacture of paper suitable for electric printing the process which consists 85 in boiling seaweed in sea-water to which carbonate of soda has been added, adding acid to the resulting liquor, then separating the supernatant liquor, adding hyposulphite of soda thereto and adding the resulting extract to paper, substantially as described. 90

4. As a new product, paper suitable for electric printing containing an extract of marine algae.

5. As a new product, paper suitable for electric printing containing an extract of seaweed. 95

6. As a new product, paper containing the extract obtained by boiling seaweed in sea-water to which carbonate of soda has been added, adding acid to the resulting liquor, and (after separating the supernatant liquor) 100 adding hyposulphite of soda thereto.

In witness whereof I have hereunto signed my name in the presence of two subscribing witnesses.

WILLIAM FRIESE-GREENE.

Witnesses:

GEORGE BELOE ELLIS,  
ROBERT MILTON SPEARPOINT.